

## 1

3,117,897

### PROCESS FOR HARDENING STEEL SHEET AND STRIPS BY OVER-AGING

Ernest Wynne Williams, Bishopston, Swansea, England, assigner to The British Iron and Steel Research Association, London, England  
No Drawing. Filed Sept. 24, 1962, Ser. No. 225,831  
Claims priority, application Great Britain Nov. 7, 1961  
8 Claims. (Cl. 148—142)

The present invention relates to a process for the annealing of cold worked steel sheet and strip and is more particularly concerned with a process for the production of plate having a hardness of at least 65 R30T units.

Steel sheet and strip is produced for the tinplate industry in a number of grades having different ranges of hardness and these grades of material are known in the British and American tinplate industries as "Temper 1," "Temper 2," etc. up to "Temper 6," the latter material being the hardest and having a hardness of 65 to 70 R30T units in the "as annealed" condition (R30T units are Rockwell hardness numbers using the superficial Rockwell tester with a 30 kg. load).

With known annealing treatments it is not possible to produce plate having the hardness required for Temper 6 from ordinary grade blackplate steels (that is low carbon steels containing less than 0.02% phosphorus), and it is at present produced from rephosphorised steels containing approximately 0.1 to 0.14% phosphorus and up to 0.14% carbon. During annealing the phosphorus goes into solid solution in the ferrite and stiffens, i.e., hardens, the product, but with a significant reduction in ductility. The presence of phosphorus also lowers the corrosion resistance of the plate and gives non-uniform mechanical properties due to the occurrence of segregation of the phosphorus content in the ingot from which the strip is rolled.

It is an object of the present invention to provide a process whereby annealed steel sheet and strip having a hardness of at least 65 R30T units can be obtained from ordinary grade, that is non-rephosphorised, blackplate steel.

Further objects and advantages of the present invention will appear from the description which follows.

According to the present invention, we provide a process for the production of annealed steel sheet and strip, which comprises heating cold worked steel sheet or strip which contains from 0.07 to 0.14% carbon and less than 0.02% phosphorus to a temperature of from 740° to 850° C., rapidly quenching the steel from this temperature to a temperature of from 150° to 250° C., and over-aging the steel within the latter temperature range whereby a stable product having a hardness of at least 65 R30T units is obtained.

The final hardness of the product after over-aging depends on the carbon content of the steel, the annealing temperature and, to a lesser extent, the quenching rate; thus in order to obtain the specified minimum hardness, it is necessary to employ a steel having a carbon content at the upper end of the specified range if an annealing temperature at the lower end of the specified range is used, or vice versa. More particularly, if an annealing temperature of from 740° to 770° C. (the

## 2

latter temperature being the Curie transition point for steel which is substantially independent of the carbon content) is used, the steel should contain from 0.12 to 0.14% carbon in order to obtain or exceed the specified minimum hardness. If annealing temperatures above the Curie point, that is from 770° to 850° C., are used, the specified minimum hardness can be obtained or exceeded with steels containing from 0.07 to 0.12% carbon.

If steels having a carbon content at the upper end of the specified range, say from 0.10 to 0.14%, are annealed at temperatures at the upper end of the specified range, say from 790° to 850° C., the final product will have a hardness greater than that of Temper 6 plate (which has a hardness of 65-70 R30T units), such a degree of hardness corresponding to that of so-called "double-reduced" tinplate. Double-reduced tinplate is produced by cold rolling tinplate after tinning so as to double its superficial area; owing to the increase in superficial area this product is much cheaper than conventional tinplate and although it has poorer properties than conventional tinplate, in respect, for example, of ductility, corrosion resistance, and uniformity of mechanical properties in the transverse and longitudinal directions with respect to the direction of rolling, the reduction in gauge is compensated by the considerable increase in hardness and stiffness and the product can be used where the service conditions are not very severe. The present invention therefore provides a method of obtaining the necessary hardness in thin tinplate of this type (of 40 to 60 pounds substance, that is 0.0044 to 0.0066 inch thickness) by heat treatment rather than by cold rolling. Such a product obtained by the present process has the advantages of greater ductility and less directionality over the product obtained by cold double reduction.

As mentioned above the hardness of the product after over-aging also depends to some extent on the quenching rate. Quenching may be effected into water or into a molten metal bath, for example a bath consisting of a 50% mixture of lead and bismuth. The faster quenching rates obtainable by water quenching enable a somewhat harder product to be obtained than when a molten metal quenching medium is used. Thus products having satisfactory Temper 6 mechanical properties (hardness 65-70 R30T units) can be obtained with steels containing from 0.08 to 0.14% carbon by quenching from the Curie point, 770° C., into water, but at the lower cooling rates associated with liquid metal quenching, the range of carbon contents which give Temper 6 hardness values using the same annealing temperature is narrowed to 0.12 to 0.14% carbon.

The steel sheet or strip is preferably heated rapidly to the annealing temperature, for example in less than 10 seconds, and is quenched immediately or after only a short holding time, i.e., less than 5 seconds. After quenching, the steel is over-aged at a temperature of from 150° to 250° C. Over-aging is preferably carried out, in the case of strip treatment, by coiling the strip as it leaves the quenching bath and holding the coil in a thermally insulated container for the required time. The period required for over-aging depends on the over-aging temperature, a longer time being required at lower temperatures and vice versa; in the middle of the temper-

ature range specified, i.e., 200° C., over-aging is normally complete in 1/2 hour. The hardness of the final product is only slightly affected by the overaging temperature; lower over-aging temperatures within the above range giving slightly harder products than higher temperatures within the range. Over-aging can be carried out in air without any appreciable oxidation taking place at temperatures below 200° C.; if over-aging is carried out at higher temperatures it is preferable to surround the steel with a non-oxidising atmosphere.

The process according to the invention is particularly suitable for the continuous high speed production of Temper 6 strip for the tinplate industry. Owing to the very short processing times of the steps which take place

200° C. for 30 to 60 minutes. Steels with the following analysis were used:

Steel W: 0.084% C; 0.31% Mn; 0.049% S; 0.018% P  
 Steel X: 0.068% C; 0.35% Mn; 0.043% S; 0.016% P  
 Steel Y: 0.11% C; 0.43% Mn; 0.035% S; 0.013% P  
 Steel A: 0.135% C; 0.46% Mn; 0.035% S; 0.010% P

(Steel A was over-aged at 230° C. for 1/2 hour, instead of at 200° C.)

10 The mechanical properties of these steels are given in Table 1 below, which also includes the results obtained with control samples of a rephosphorised steel annealed commercially by a known process and then temper rolled and heat treated as described above:

Table 1

| Steel                                  | As annealed,<br>R30T | As temper rolled |                  | After strain aging 200° C./30<br>min. |                  |                 | Thickness,<br>ins. |
|----------------------------------------|----------------------|------------------|------------------|---------------------------------------|------------------|-----------------|--------------------|
|                                        |                      | R30T             | Erichsen,<br>mm. | R30T                                  | Erichsen,<br>mm. | Jenkins<br>Bend |                    |
| W-----                                 | 67.3                 | 68.7             | 6.35             | 73.1                                  | 5.55             | 9/6             | .0135              |
| X-----                                 | 66.1                 | 68.3             | 7.0              | 72.2                                  | 6.2              | 11/6            | .012               |
| Y-----                                 | 69.2                 | 70.7             | 6.4              | 74.1                                  | 5.2              | 10 1/4/7 1/2    | .0115              |
| Commercial<br>rephosphor-<br>ised----- | 64.7                 | 67.0             | 7.55             | 70.8                                  | 6.6              | 12/8            | .0135              |
| A-----                                 | 7.10                 | 71.2             | 7.35             | 74.6                                  | 5.95             | 12/7            | .0135              |

in-line, namely up to 10 seconds for heating to the annealing temperature, not more than 5 seconds hold at this temperature, and about 5 seconds for quenching before the strip is coiled, the process can be operated continuously at high speed in plant which costs a fraction of that for the continuous high speed production of Temper 6 plate by present methods, and which occupies a fraction of the space required for the latter.

In order that the invention may be more fully understood, the following examples are given by way of illustration only:

#### EXAMPLE 1

Samples 4 1/2 in. x 6 in. of cold worked steel sheet having different carbon contents were heated linearly in a high frequency electrical induction heater to 770° C. in 7 1/2 seconds, this temperature was held for 1 1/2 seconds, and the samples were then quenched in water. The samples were then over-aged at 200° C. for 1/2 hour. The carbon content of the samples and the hardness of the samples (in R30T units) after over-aging were as follows:

|                |      |
|----------------|------|
| 0.135% C ----- | 71.9 |
| 0.11% C -----  | 69.7 |
| 0.10% C -----  | 68.9 |
| 0.09% C -----  | 66.8 |
| 0.076% C ----- | 66   |

#### EXAMPLE 2

Samples 4 1/2 in. x 6 in. of cold worked steel sheet having different carbon contents were annealed under the conditions described in Example 1. After over-aging, the samples were temper rolled on a 6 in. mill with smooth rolls to 2 1/4-2 3/4 extension and were then given a simulated lacquer stoving treatment by being maintained at

40

45

50

55

60

65

70

75

#### EXAMPLE 3

Samples of cold worked steel sheet having different carbon contents were induction heated to the Curie point (770° C.) and quenched into a molten metal quenching bath consisting of 50% lead-50% bismuth. Two heating cycles, namely heating to 770° C. in 5 seconds with 5 seconds hold (1st heating cycle) and to 770° C. in 3 seconds with 1 second hold (2nd heating cycle) were used; two bath temperatures, 160° C. and 200° C. were used in conjunction with the 1st heating cycle and a bath temperature of 200° C. was used in conjunction with the 2nd heating cycle. Each sample was over-aged by being left in the bath for 30 minutes after quenching.

The hardness of the annealed samples (in R30T units) is set out in Table 2 below:

Table 2

| Carbon content, percent | 1st heating cycle    |                      | 2nd heating cycle    |
|-------------------------|----------------------|----------------------|----------------------|
|                         | Quench to<br>160° C. | Quench to<br>200° C. | Quench to<br>200° C. |
| 0.12-----               | 69.1                 | 67.5                 | 66.5                 |
| 0.135-----              | 72.4                 | 70.0                 | 69.5                 |

#### EXAMPLE 4

Samples of cold worked steel sheet having different carbon contents were heated to temperatures between 740° C. and 830° C. by immersion for 20 seconds in a salt bath maintained at the temperature in question, then quenched into a 50% lead-50% bismuth bath maintained at 200° C. and held over at the latter temperature for 30 minutes.

The results of tests made on the samples after this treatment, together with an analysis of the principal con-

stituents of the steels other than iron, are given in Table 3 below:

equivalent to a heating time of 15 seconds and a holding time of 5 seconds).

Table 3

| Annealing temperature, ° C. | 740             | 750            | 755            | 760            | 770            | 775           | 780                  |
|-----------------------------|-----------------|----------------|----------------|----------------|----------------|---------------|----------------------|
| <b>Steel analysis:</b>      |                 |                |                |                |                |               |                      |
| .05C; .38 Mn; .022S; .010P  | 56<br>21/19½    | 56.5<br>21/19½ | 6.95<br>60.5   | 56.5<br>61.1   | -----          | -----         | 64.0<br>7.6          |
| .07C; .40 Mn; .033S; .013P  | 7.1<br>17/14    | 6.7<br>17/14   | -----<br>63.6  | 8.05<br>16½/14 | -----          | -----         | 18/14<br>65.6        |
| .10C; .44 Mn; .020S; .014P  | 60.5<br>6.8     | 62<br>17/11½   | -----<br>7.95  | 63.6<br>13½/9  | -----          | -----         | 7.5<br>14/10         |
| .10C; .67 Mn; .018S; .012P  | 6.8<br>63.5     | 6.45<br>8/7    | 65<br>6.4      | 66<br>7.0      | -----          | -----         | 67.5<br>6.1          |
| .113C; .45 Mn; .019S; .008P | 6.8<br>14½/9½   | 6.45<br>14/8   | 68.5<br>71.4   | 68.5<br>7.2    | -----          | -----         | 71.4<br>6.7          |
| .14C; .49 Mn; .026S; .009P  | 66.5<br>13½/9½  | 68.5<br>15/8   | 71.4<br>7.3    | 71.4<br>14/8   | -----          | -----         | 11/8<br>75.2<br>6.35 |
| .077C                       | -----           | 64.4<br>7.55   | -----          | -----          | 67.1<br>7.9    | 67.5<br>7.9   | -----                |
| .099C                       | -----           | 15½/13<br>64.3 | 7.5            | -----          | 16/14½<br>67.2 | 18/12<br>7.85 | -----                |
| .126C; .46 Mn; .030S; .011P | 64.5<br>13½/10½ | 66.5<br>13½/10 | 67.8<br>13½/10 | 68.6<br>7.8    | 68.6<br>12/7½  | 70.5<br>8.2   | 12/7½                |
| Annealing temperature, ° C. | 785             | 790            | 795            | 800            | 805            | 810           | 830                  |
| <b>Steel analysis:</b>      |                 |                |                |                |                |               |                      |
| .05C; .38 Mn; .022S; .010P  | 62<br>21/19½    | 6.9<br>64.3    | -----          | -----          | 60<br>67.8     | -----         | 73.1<br>6.2          |
| .07C; .40 Mn; .033S; .013P  | 7.55<br>17/14   | 7.55<br>69.5   | -----<br>6.5   | 71.3<br>6.25   | 73.4<br>5.45   | 15/9<br>9/6   | -----                |
| .10C; .44 Mn; .020S; .014P  | 11/6<br>70.5    | 11/6<br>70.5   | 11/6<br>7.5    | 72.1<br>5.1    | 77.0<br>4.3    | 77.0<br>5/3   | 5/3                  |
| .10C; .67 Mn; .018S; .012P  | 5.1<br>8/6      | 5.1<br>8/6     | 73.7<br>6.6    | 73.7<br>6.6    | 79.2<br>6.45   | 79.2<br>5/3   | -----                |
| .113C; .45 Mn; .019S; .008P | 10/7<br>73.6    | 10/7<br>73.6   | 10/7<br>6.5    | 10/7<br>6.5    | -----          | -----         | 5/3                  |
| .14C; .49 Mn; .026S; .009P  | 67.3<br>7.95    | 67.3<br>7.95   | 68.2<br>7.65   | 68.2<br>7.65   | 73.8<br>5.5    | 73.8<br>5.5   | -----                |
| .077C                       | -----           | 7.95<br>13/9   | 7.95<br>13/9   | 70.5<br>69.3   | 70.9<br>7.55   | 77.3<br>4.2   | 8/6                  |
| .099C                       | -----           | 7.8<br>18/12   | 7.8<br>18/12   | 7.8<br>17/11   | 7.8<br>14/8    | 80.9<br>9/7   | -----                |
| .126C; .46 Mn; .030S; .011P | 11½/6<br>73.6   | 11½/6<br>73.6  | 11½/6<br>6.5   | 11½/6<br>6.5   | -----          | 5.95<br>8/6   | -----                |

NOTE.—The properties presented are in each case (reading downwards) Hardness (R30T), Erichsen (mm.) and Jenkins Bend values.

It will be seen from these results that there is a consistent increase of hardness with annealing temperatures.

## EXAMPLE 5

60

Small samples 2 inches x 1 inch of cold worked steel sheet having different carbon contents were heated rapidly in an electric induction heater to 770° C. with thermocouple wires spot welded to each sample and connected to a 1/4 second f.s.d. recorder. The samples were heated to and held at the annealing temperature for different times. They were quenched into a 50% lead-50% bismuth bath maintained at 200° C. and aged at the latter temperature for 30 minutes.

The hardness values of the samples after this treatment are given in Table 4 below, together with the comparative values for similar samples which had been heated to the same annealing temperature (770° C.) in a salt bath by immersion therein for 20 seconds (estimated as being 75

Table 4

|     | Carbon content percent | Heating time to 770° C., secs. | Holding time at 770° C., secs. | Hardness R30T |
|-----|------------------------|--------------------------------|--------------------------------|---------------|
| .14 | 0.5                    | 0.5                            | 0.5                            | 71.6          |
|     | 1                      | 0.5                            | 0.5                            | 71.3          |
|     | 3                      | 0                              | 0                              | 71.3          |
|     | 3                      | 5                              | 5                              | 73.5          |
|     | 3                      | 10                             | 10                             | 74.4          |
|     | 1 15                   | 1 5                            | 1 5                            | 2 73.5        |
| .10 | 0.5                    | 0.5                            | 0.5                            | 69.5          |
|     | 3                      | 0                              | 0                              | 68.2          |
|     | 3                      | 5                              | 5                              | 68.1          |
|     | 3                      | 10                             | 10                             | 69.8          |
|     | 1 15                   | 1 5                            | 1 5                            | 2 68.5        |
|     | 0.5                    | 0.5                            | 0.5                            | 66.4          |
| .07 | 1                      | 0.5                            | 0.5                            | 65.6          |
|     | 3                      | 0                              | 0                              | 63.7          |
|     | 3                      | 5                              | 5                              | 64.2          |
|     | 3                      | 10                             | 10                             | 63.9          |
|     | 1 15                   | 1 5                            | 1 5                            | 2 63.0        |
|     |                        |                                |                                |               |

<sup>1</sup> Est.<sup>2</sup> Salt bath.

It will be seen from these results that the heating rate has little effect upon the hardness obtained with steel containing 0.10% carbon, while with the 0.14% carbon steel, fast heating rates give somewhat lower hardness values than salt bath heating and with the 0.07% carbon steel, fast heating rates give somewhat higher values.

#### EXAMPLE 6

In order to demonstrate the effect of different quenching rates, samples of 0.077% carbon cold worked steel

and aging temperatures on hardness values was also ascertained by heating samples of cold worked steel sheet having different carbon contents in an electric induction heater to 770° C., the heating time being respectively 1 second, 5 seconds or 10 seconds, quenching the samples into 50% lead-50% bismuth baths respectively maintained at 150° C. or 200° C., and over-aging the samples at 150° C. for 3/4 hour or 200° C. for 1/2 hour.

The hardness values obtained are set out in Table 6 below:

Table 6

| Carbon content, percent | 1 sec. heating to 770° C.                     |                                               | 5 sec. heating to 770° C.                     |                                               |                                               | 10 sec. heating to 770° C.                    |                                               |
|-------------------------|-----------------------------------------------|-----------------------------------------------|-----------------------------------------------|-----------------------------------------------|-----------------------------------------------|-----------------------------------------------|-----------------------------------------------|
|                         | Quench to 150° C. overage at 150° C., 3/4 hr. | Quench to 200° C. overage at 200° C., 1/2 hr. | Quench to 150° C. overage at 150° C., 3/4 hr. | Quench to 200° C. overage at 150° C., 3/4 hr. | Quench to 200° C. overage at 200° C., 1/2 hr. | Quench to 150° C. overage at 150° C., 3/4 hr. | Quench to 200° C. overage at 200° C., 1/2 hr. |
|                         | R30T                                          | R30T                                          | R30T                                          | R30T                                          | R30T                                          | R30T                                          | R30T                                          |
| 0.071                   | 66.2                                          | 65.1                                          | 64.8                                          | 64.0                                          | 63.2                                          | 65.0                                          | 63.5                                          |
| 0.087                   | 68.5                                          | 66.0                                          | 67.3                                          | 66.2                                          | 65.9                                          | 67.7                                          | 65.5                                          |
| 0.104                   | 71.7                                          | 71.2                                          | 72.6                                          | 70.5                                          | 69.5                                          | 71.7                                          | 70.1                                          |
| 0.109                   | 73.3                                          | 72.4                                          | 72.9                                          | 71.8                                          | 70.4                                          | 73.0                                          | 70.6                                          |

sheet was heated to 810° C. in a salt bath, quenched into 50% lead-50% bismuth baths maintained at 200° C., 250° C. and 350° C. respectively and held in the baths for 30 minutes. In addition some of the samples were quenched into the baths at 350° C. and 250° C. and then immediately transferred to other baths for holding at lower temperatures.

The results obtained by these treatments are given in Table 5 below:

Table 5

| Holding temperature      | 350° C. |        |       | 250° C. |        |           | 200° C. |        |               |
|--------------------------|---------|--------|-------|---------|--------|-----------|---------|--------|---------------|
|                          | R30T    | E(mm.) | J.B.  | R30T    | E(mm.) | J.B.      | R30T    | E(mm.) | J.B.          |
| Quench bath temperature: |         |        |       |         |        |           |         |        |               |
| 350° C.                  | 59.9    | 7.35   | 18/16 | 60.7    | 7.05   | 18/15     | 61.0    | 7.35   | 18 1/2/14     |
| 250° C.                  |         |        |       | 60.4    | 7.3    | 17 1/2/16 | 62.6    | 6.7    | 18 1/2/14 1/2 |
| 200° C.                  |         |        |       |         |        |           | 67.8    | 6.8    | 16/13         |

It will be seen that with steels having the low carbon content (0.077%) of the samples used in these treatments, the minimum hardness for Temper 6 material (65 R30T units) was only obtained with a quench bath temperature and holding temperature of 200° C., higher quench bath and holding temperature (and therefore slower cooling rates from the annealing temperature) not enabling this minimum hardness value to be obtained.

50 thickness of 0.0065 inch. The cold reduced samples were then heated to 810° C. by immersion for 4 seconds in a salt bath, quenched into a 50% lead-50% bismuth bath maintained at 150° C. and held at the latter temperature for 45 minutes. After this treatment, some of the samples were temper rolled to give a 2 1/2% reduction and strain aged at 350° C. for 20 seconds.

The results obtained are set out in Table 7 below:

Table 7

| Carbon content, percent | Thickness, ins. | "An annealed" (Quenched from 810° C. to 150° C.) |                   |        |       | As temper rolled and strain aged |                   |        |        |
|-------------------------|-----------------|--------------------------------------------------|-------------------|--------|-------|----------------------------------|-------------------|--------|--------|
|                         |                 | R15T                                             | R30T <sup>1</sup> | E(mm.) | J.B.  | R15T                             | R30T <sup>1</sup> | E(mm.) | J.B.   |
| 0.05                    | 0.0064          | 82.5                                             | 61.5              | 5.35   | 43/33 |                                  |                   |        |        |
| 0.07                    | 0.0063          | 87.3                                             | 71.5              | 4.7    | 41/29 |                                  |                   |        |        |
| 0.105                   | 0.0063          | 83.0                                             | 73.0              | 4.5    | 26/15 | 89.5                             | 75.5              | 5.0    | 25/15  |
| 0.115                   | 0.0065          | 83.0                                             | 73.0              | 4.3    | 28/26 | 89.5                             | 75.5              | 4.6    | 25/14  |
| 0.125                   | 0.0063          | 83.5                                             | 74.0              | 4.55   | 20/13 | 90.5                             | 77.5              | 4.7    | 14 8/2 |

<sup>1</sup> The R30T values are converted R15T values (Wilson conversion chart).

The results obtained also show that the effect of different holding temperatures on the properties obtained after quenching to 350° C. and 250° C. is not very great, but the effect of quenching temperature itself is considerable, especially over the range 250° to 200° C.

#### EXAMPLE 7

The effect of different heating rates, quenching rates

70 and the hardness of the treated samples containing 0.105% or more carbon is comparable to that of so-called "double-reduced" tinplate, that is tinplate of 40 to 60 pound substance (corresponding to a thickness of 0.0044 to 0.0066 inch), but the ductility is greater and the directionality less, than that of double reduced tinplate (a typical example of the latter having Erichsen value of 3.0 mm. and Jenkins bend value of 25-1/2/7).

## EXAMPLE 9

Samples (12 inches x 5 inches) of cold reduced steel sheet having a carbon content of 0.14% were heated in a high frequency induction heater to 770° C., quenched in water, and aged at 200° C. for 30 minutes. The samples were then pickled, temper rolled to give a 2½% reduction on a laboratory mill, electrolytically tinned, flow brightened, stoved at 200° C. for 45 minutes, and then stamped into standard beer can ends for double seaming and end peaking tests.

The hardness of the stoved samples (75 R30T units) was slightly higher than the specified limit for Temper 6 plate, but no failures occurred during double seam forming. Can peaking pressure values were, on average, 10% greater than the minimum requirement for beer cans and 12% greater than for cans made using a commercial rephosphorised steel of the same gauge, temper rolled under identical conditions. The average Erichsen and Jenkins bend values for the finished samples were 6.1 mm. and 9-1/2/5-1/2 respectively.

## EXAMPLE 10

Cold reduced steel strip 5 inches wide and containing 0.12% carbon, 0.035% sulphur, 0.010% phosphorus and 0.48% manganese was passed through a continuous annealing plant at approximately 150 feet/minute. In this plant the strip was heated to an annealing temperature of 780° C. in approximately 3 seconds and then quenched to 200° C. in a molten 50% lead-50% bismuth bath. The strip was coiled as it came from the quench bath and was maintained in the coil at 200° C. for 30 minutes.

The strip was then temper rolled to 2½% extension using shot blasted and smooth rolls and then electrolytically tinned (4 oz. deposit) and flow brightened on a continuous electrolytic tinning line.

The tinned and flow brightening strip was then subjected to a lacquer stoving treatment before being tested. The average results of these tests together with probable values of a commercial rephosphorised Temper 6 plate are given in Table 8 below:

Table 8

| Samples                  | Hardness | Erichsen | Jenkins Bends | Plate substance lb./basis box | Schopper values, kg./sq. mm. |             |              |             | Average peaking pressure, percentage of min. requirements (corrected to 114 lb. substance) |  |
|--------------------------|----------|----------|---------------|-------------------------------|------------------------------|-------------|--------------|-------------|--------------------------------------------------------------------------------------------|--|
|                          |          |          |               |                               | With grain                   |             | Across grain |             |                                                                                            |  |
|                          |          |          |               |                               | Yld. pt.                     | Load at 90° | Yld. pt.     | Load at 90° |                                                                                            |  |
| Experimental tinplate... | 69-71    | 5.4-5.8  | 15/10         | 111-116                       | 45.5                         | 57.5        | 50           | 63          | 103                                                                                        |  |
| Commercial tinplate...   | 69-70    | 5.9      | 11/6          | 114-118                       | 42                           | 54          | 45           | 67          | 102.5                                                                                      |  |

No difficulties were experienced during stamping and double seaming of the can ends and experimental tinplate compared favourably with rephosphorised steel. The only significant difference in behaviour was found in the bend test results where the experimental material exhibited less directionality and higher values than the commercial material.

I claim:

1. A process for the production of annealed steel sheet and strip, which comprises the steps of heating cold worked steel sheet or strip which contains from 0.07 to 0.14% carbon and less than 0.02% phosphorus to a temperature of from 740° to 850° C., rapidly quenching the steel from this temperature to a temperature of from 150° to 250° C., and then over-aging the steel within the latter temperature range until a stable product having a hardness of at least 65 R30T units is obtained.

2. A process according to claim 1, wherein the steel is quenched into a molten metal bath.

3. A process for the production of annealed steel sheet and strip, which comprises the steps of heating cold worked steel sheet or strip which contains from 0.12 to 0.14% carbon and less than 0.02% phosphorus to a temperature of from 740° to 770° C., rapidly quenching the steel from this temperature to a temperature of from 150° to 250° C., and then over-aging the steel within the latter temperature range until a stable product having a hardness of at least 65 R30T units is obtained.

4. A process for the production of annealed steel sheet or strip, which comprises the steps of heating cold worked steel sheet or strip which contains from 0.07 to 0.12% carbon and less than 0.02% phosphorus to a temperature of from 770° to 850° C., rapidly quenching the steel from this temperature to a temperature of from 150° to 250° C., and then over-aging the steel within the latter temperature range until a stable product having a hardness of at least 65 R30T units is obtained.

5. A process for the production of annealed steel sheet and strip, which comprises the steps of rapidly heating cold worked steel sheet or strip which contains from 0.07 to 0.14% carbon and less than 0.02% phosphorus in less than 10 seconds to a temperature of from 740° to 850° C., holding the steel at said temperature for less than 5 seconds, rapidly quenching the steel from said temperature to a temperature of from 150° to 250° C., and over-aging the steel within the latter temperature range for a period of about 30 minutes until a stable product having a hardness of at least 65 R30T units is obtained.

6. A process according to claim 5, wherein said steel is quenched into a 50% lead-50% bismuth bath.

7. A continuous process for the production of annealed steel strip, which comprises the steps of continuously passing cold rolled steel strip which contains from 0.07 to 0.14% carbon and less than 0.02% phosphorus through a heating zone wherein said strip is heated to a temperature of from 740° to 850° C. in less than 10 seconds, continuously passing the heated strip to a quench bath wherein it is quenched to a temperature of from 150° to 250° C., coiling the strip, and maintaining the

55 strip in the coil at a temperature of from 150° to 250° C. for about 30 minutes until a stable product having a hardness of at least 65 R30T units is obtained.

8. A process according to claim 7, wherein the quench bath consists of a 50% lead-50% bismuth mixture.

## References Cited in the file of this patent

## UNITED STATES PATENTS

2,387,919      Lose \_\_\_\_\_ Oct. 30, 1945

65                   OTHER REFERENCES

A.S.M. Metals Handbook (1948 Ed.), published by the Amer. Soc. for Metals, Cleveland, Ohio. (Pages 439, 309, and 744 relied on.)

70                   A.S.M. Trans. "The Effect of Subboundaries and Carbide Distribution of the Notch Toughness of an Ingot Iron," by J. C. Danko and R. D. Stout (1956). Reprint No. 5. Pages 5-2 relied on.